



US006140035A

# United States Patent [19]

Klingman et al.

[11] Patent Number: 6,140,035

[45] Date of Patent: \*Oct. 31, 2000

[54] **PHOTOGRAPHIC ELEMENT COMPRISING A MIXTURE OF SENSITIZING DYES**

[75] Inventors: **Karen J. Klingman**, Pittsford; **Bruce E. Kahn**, Rochester; **Richard L. Parton**, Webster; **Thomas R. Dobles**, Hilton; **David A. Stegman**, Churchville, all of N.Y.; **Teresa A. Smith**, Belmont, Mass.; **John D. Lewis**, Webster, N.Y.

[73] Assignee: **Eastman Kodak Company**, Rochester, N.Y.

[\*] Notice: This patent is subject to a terminal disclaimer.

[21] Appl. No.: 09/151,123

[22] Filed: Sep. 10, 1998

[51] Int. Cl.<sup>7</sup> G03C 1/09; G03C 1/16; G03C 1/29

[52] U.S. Cl. 430/574

[58] Field of Search 430/572, 574, 430/583, 613, 605

## [56] References Cited

### U.S. PATENT DOCUMENTS

- |           |         |                    |
|-----------|---------|--------------------|
| 3,672,898 | 6/1972  | Schwan et al. .    |
| 4,378,424 | 3/1983  | Altland et al. .   |
| 4,439,520 | 3/1984  | Kofron et al. .    |
| 4,469,785 | 9/1984  | Tanaka et al. .    |
| 4,518,689 | 5/1985  | Noguchi et al. .   |
| 4,925,780 | 5/1990  | Yoshizawa et al. . |
| 4,939,078 | 7/1990  | Kuramoto et al. .  |
| 5,013,642 | 5/1991  | Muenter et al. .   |
| 5,047,311 | 9/1991  | Endo et al. .      |
| 5,049,485 | 9/1991  | Deaton .           |
| 5,368,996 | 11/1994 | Asami .            |
| 5,418,126 | 5/1995  | Stegman et al. .   |
| 5,418,127 | 5/1995  | Budz et al. .      |
| 5,474,887 | 12/1995 | Reed et al. .      |
| 5,538,836 | 7/1996  | Ueda et al. .      |
| 5,582,960 | 12/1996 | Nielsen et al. .   |

### OTHER PUBLICATIONS

*The Theory of the Photographic Process*, T.H. James, ed.,

4th edition, Macmillan, N.Y. 1977, p. 265.

Y. Yonezawa, T. Miyama, and H. Ishizawa, *J. Imaging Sci. Technol.*, 39 331(1995).

V. Bliznyuk and H. Mohwald, *Thin Solid Films*, 261 275 (1995).

L. Penner and D. Mobius, *Thin Solid Films*, 132 185 (1985).

G. Scheibe, A. Mareis, H. Ecker, *Naturwiss.*, 29 474(1937).

Primary Examiner—Thorl Chea  
Attorney, Agent, or Firm—Edith A. Rice

## [57] ABSTRACT

A photographic element comprises at least one silver halide emulsion layer in which:

a) the silver halide has been spectrally sensitized with a first blue sensitizing dye having a  $\lambda_1$  less than or equal to about 475 nm and a second blue sensitizing dye having a  $\lambda_2$ , wherein the following relationship is met:

$$0.12 \text{ (eV)} \geq 1.25 \frac{(\text{nm})}{(\text{eV})} \times 10^3 \left( \frac{1}{\lambda_2(\text{nm})} - \frac{1}{\lambda_1(\text{nm})} \right)$$

wherein  $\lambda_1$  is the wavelength in nanometers (nm) of maximum absorption of a silver halide emulsion sensitized with the first dye and  $\lambda_2$  is the wavelength of maximum absorption of a silver halide emulsion sensitized with the second dye, with the proviso that neither the first nor the second dye contains selenium. The silver halide emulsion of said layer is chemically sensitized with a gold(I) compound and preferably with the combination of a gold compound and a disulfide compound; and

b) the silver halide has been chemically sensitized with a gold compound of formula (I):



wherein

L is a mesoionic compound;

X is an anion; and

$\text{L}^1$  is a Lewis donor ligand.

19 Claims, No Drawings

## 1

**PHOTOGRAPHIC ELEMENT COMPRISING  
A MIXTURE OF SENSITIZING DYES**

**FIELD OF THE INVENTION**

This invention relates to a photographic element, in particular to a photographic element comprising a silver halide emulsion layer containing at least two sensitizing dyes.

**BACKGROUND OF THE INVENTION**

Photographic elements typically contain a light sensitive silver halide emulsion layer sensitive to blue light. A sensitizing dye is generally used to provide the desired sensitivity to blue light. Dyes used for this purpose tend to be water insoluble and are added to a silver halide emulsion in a water/alcohol solution. A problem that arises with this procedure is crystallization of the dye. Because of this, larger amounts of dye must be used to ensure the desired degree of sensitivity. Also crystallization of the dye poses difficulties in manufacture of photographic elements, e.g., plugging filters used to purify the emulsion prior to coating the emulsion on a support.

In the manufacture of photographic elements, the components used can result in undesirable results. For example, it is known to use certain gold compounds. However certain gold compounds react with gelatin which results in variability from batch to batch. Also, it is known to chemically sensitize silver halide using a gold compound that also contains sulfur. This limits the relative amounts of gold and sulfur to the stoichiometric amounts of the compound. It is desirable to vary the amount of gold versus sulfur to obtain the optimum sensitization for a particular photographic use.

**PROBLEM TO BE SOLVED BY THE  
INVENTION**

This invention addresses the problems encountered in the manufacture of a photographic element, in particular, the problems of crystallization of the sensitizing dye, reaction of the gold compound with gelatin and optimizing the relative amounts of gold and sulfur used to chemically sensitize the silver halide.

**SUMMARY OF THE INVENTION**

We have discovered that the selection of appropriate sensitizing agents (both spectral and chemical sensitization) avoids the problems of the prior art.

One aspect of this invention comprises a photographic element comprising at least one silver halide emulsion layer in which:

- a) the silver halide has been sensitized with a first blue sensitizing dye having a  $\lambda_1$  less than or equal to about 475 nm and a second blue sensitizing dye having a  $\lambda_2$ , wherein wherein  $\lambda_1$  is longer than  $\lambda_2$  and  $\lambda_1$  and  $\lambda_2$  are separated by an energy gap,  $\Delta E$ , which does not exceed 0.12 eV, where  $\Delta E$  is defined by the following equation:

$$\Delta E = 1.25 \frac{(\text{nm})}{(\text{eV})} \times 10^3 \left( \frac{1}{\lambda_2(\text{nm})} - \frac{1}{\lambda_1(\text{nm})} \right) \leq 12.0 \text{ (eV)}$$

## 2

wherein  $\lambda_1$  is the wavelength in nanometers (nm) of maximum absorption of a silver halide emulsion sensitized with the long dye and  $\lambda_2$  is the wavelength of maximum absorption of a silver halide emulsion sensitized with the short dye, 5 with the proviso that neither the first nor the second dye contains selenium; and

- b) the silver halide has been chemically sensitized with a gold(I) compound of formula (I)

10



wherein

L is a mesoionic compound;

X is an anion; and

$\text{L}^1$  is a Lewis donor ligand.

In preferred embodiments of the invention the emulsion layer further comprises a disulfide compound of formula (II):



35 wherein:

X' is independently —O—, —NH— or —NR—, where R is an alkyl group, a fluoroalkyl group, an aryl group or a sulfonyl group;

m and r are independently 0, 1 or 2, with the proviso that 40 m and r are not both 0;

M is —H or a cationic species;

Ar is an aromatic group; and

$\text{L}^2$  is a linking group, where p is 1.

45 The photographic element may contain one or more additional blue sensitizing dyes.

**ADVANTAGEOUS EFFECT OF THE  
INVENTION**

50 This invention: (1) provides an adjustable sensitization envelope by the appropriate selection of the first and second dyes; (2) provides adjustable gold/sulfur chemical sensitization by use of appropriate amounts of a gold compound of formula (I) and a disulfide compound of formula (II) and (3) provides improved manufacturability.

**DETAILED DESCRIPTION OF THE  
INVENTION**

60 In our invention a silver halide emulsion is spectrally sensitized to blue light using a combination of two blue dyes. Preferred dyes are of the following classes:

TABLE A

| <u>The General Series of Blue Chromophores Under Consideration</u> |                       |           |
|--------------------------------------------------------------------|-----------------------|-----------|
| Dye Structure                                                      | Peak Wave-length (nm) | Dye Class |
|                                                                    | 470 nm                | Class F   |
|                                                                    | 450 nm                | Class E   |
|                                                                    | 450 nm                | Class E'  |
|                                                                    | 440 nm                | Class D   |
|                                                                    | 430 nm                | Class C   |
|                                                                    | 420 nm                | Class B   |
|                                                                    | 410 nm                | Class A   |

wherein  $Z_1$ ,  $Z_2$  and  $Z''$  are independently a hydrogen or halogen atom or a substituted or unsubstituted alkyl, substituted or unsubstituted alkoxy, substituted or unsubstituted aromatic, substituted or unsubstituted alkoxy carbonyl or substituted or unsubstituted heterocyclic group; and  $R_1$  and  $R_2$ , are independently substituted or unsubstituted alkyl,

substituted or unsubstituted alkenyl or substituted or unsubstituted aryl. In preferred embodiments of the invention, at least one of  $R_1$  and  $R_2$ , contains a water solubilizing group, such as sulfoalkyl, carboxyalkyl, sulfoaryl and the like. The dyes may also contain one or more substituents in other positions of the benzo ring. <sup>65</sup>

The approximate peak wavelength for each of the parent chromophores, when optimally substituted to enable aggregation, is shown. In general, we designate the pair of dyes which comprise the mixed aggregate as comprising a "long dye" and a "short dye" (i.e. dyes corresponding to the first and second dyes, respectively). Proceeding from top to bottom of Table A, adjacent pairs of long and short dyes will, when optimally substituted, form mixed aggregates. That is, a dye with a maximum peak wavelength of about 470 nm will form a mixed aggregate with a dye with a maximum peak wavelength of about 450 nm or greater, a dye with a maximum peak wavelength of about 450 nm will form a mixed aggregate with a dye with a peak wavelength of about 440 nm or greater, and so on down to a dye with a maximum peak wavelength of about 420 nm will form a mixed aggregate with a dye with a maximum peak wavelength of about 410 nm or greater. In the blue region of the spectrum the differences in wavelengths between the short and long dyes determined by a  $\Delta E$  that does not exceed 0.12 eV will range from about 15 nm to about 25 nm. Dyes need not be of different classes. For example, it has been found that a dye at the high end of the wavelength range for dyes of that class can be advantageously used with a dye at the low end of the wavelength range. For example a dye of class F having a peak wavelength of about 470 nm can be paired with a dye of class F having a peak wavelength of about 465 nm or less (not exceeding 0.12 eV).

The following Table A' provides a correlation between of the peak absorption wavelength of the long dye and the peak absorption wavelength of the the short dye such that the peak absorption wavelength between the two dyes does not exceed 0.12 eV.

TABLE A'

| Long dye wavelength in nm | Short dye wavelength in nm | 35 |
|---------------------------|----------------------------|----|
| 400                       | 385.2                      |    |
| 401                       | 386.1                      |    |
| 402                       | 387.1                      |    |
| 403                       | 388.0                      |    |
| 404                       | 388.9                      | 40 |
| 405                       | 389.8                      |    |
| 406                       | 390.8                      |    |
| 407                       | 391.7                      |    |
| 408                       | 392.6                      |    |
| 409                       | 393.5                      |    |
| 410                       | 394.5                      | 45 |
| 411                       | 395.4                      |    |
| 412                       | 396.3                      |    |
| 413                       | 397.2                      |    |
| 414                       | 398.2                      |    |
| 415                       | 399.1                      |    |
| 416                       | 400.0                      | 50 |
| 417                       | 400.9                      |    |
| 418                       | 401.9                      |    |
| 419                       | 402.8                      |    |
| 420                       | 403.7                      |    |
| 421                       | 404.6                      |    |
| 422                       | 405.6                      | 55 |
| 423                       | 406.5                      |    |
| 424                       | 407.4                      |    |
| 425                       | 408.3                      |    |
| 426                       | 409.3                      |    |
| 427                       | 410.2                      |    |
| 428                       | 411.1                      |    |
| 429                       | 412.0                      |    |
| 430                       | 413.0                      |    |
| 431                       | 413.9                      |    |
| 432                       | 414.8                      |    |
| 433                       | 415.7                      |    |
| 434                       | 416.6                      |    |
| 435                       | 417.6                      |    |
| 436                       | 418.5                      |    |

TABLE A'-continued

| Long dye wavelength in nm | Short dye wavelength in nm |
|---------------------------|----------------------------|
| 437                       | 419.4                      |
| 438                       | 420.3                      |
| 439                       | 421.2                      |
| 440                       | 422.2                      |
| 441                       | 423.1                      |
| 442                       | 424.0                      |
| 443                       | 424.9                      |
| 444                       | 425.8                      |
| 445                       | 426.8                      |
| 446                       | 427.7                      |
| 447                       | 428.6                      |
| 448                       | 429.5                      |
| 449                       | 430.4                      |
| 450                       | 431.4                      |
| 451                       | 432.3                      |
| 452                       | 433.2                      |
| 453                       | 434.1                      |
| 454                       | 435.0                      |
| 455                       | 436.0                      |
| 456                       | 436.9                      |
| 457                       | 437.8                      |
| 458                       | 438.7                      |
| 459                       | 439.6                      |
| 460                       | 440.5                      |
| 461                       | 441.5                      |
| 462                       | 442.4                      |
| 463                       | 443.3                      |
| 464                       | 444.2                      |
| 465                       | 445.1                      |
| 466                       | 446.0                      |
| 467                       | 447.0                      |
| 468                       | 447.9                      |
| 469                       | 448.8                      |
| 470                       | 449.7                      |
| 471                       | 450.6                      |
| 472                       | 451.5                      |
| 473                       | 452.5                      |
| 474                       | 453.4                      |
| 475                       | 454.3                      |
| 476                       | 455.2                      |
| 477                       | 456.1                      |
| 478                       | 457.0                      |
| 479                       | 457.9                      |
| 480                       | 458.9                      |
| 481                       | 459.8                      |
| 482                       | 460.7                      |
| 483                       | 461.6                      |
| 484                       | 462.5                      |
| 485                       | 463.4                      |
| 486                       | 464.3                      |
| 487                       | 465.2                      |
| 488                       | 466.2                      |
| 489                       | 467.1                      |
| 490                       | 468.0                      |
| 491                       | 468.9                      |
| 492                       | 469.8                      |
| 493                       | 470.7                      |
| 494                       | 471.6                      |
| 495                       | 472.5                      |
| 496                       | 473.5                      |
| 497                       | 474.4                      |
| 498                       | 475.3                      |
| 499                       | 476.2                      |
| 500                       | 477.1                      |

As mentioned above, the dyes should be J-aggregating dyes which form a mixed aggregate when used in combination. As is well-known in the art, a very wide variety of substituents may be used to effect J-aggregation on predominantly AgBr emulsions. When the dye is an oxacyanine, thiacyanine, oxacarbocyanine, or thiacarbocyanine, there are abundant literature examples of aggregating cyanine dyes which contain lower alkyl, halo, lower alkoxy, aromatic and heterocyclic substituents.

When reference in this application is made to a particular moiety as a "group", this means that the moiety may itself

be unsubstituted or substituted with one or more substituents. For example, "alkyl group" refers to a substituted or unsubstituted alkyl, alkoxy refers to a substituted or unsubstituted alkoxy group, "aromatic substituent" refers to a substituted or unsubstituted aromatic group and "heterocyclic substituent" refers to a substituted or unsubstituted heterocyclic group. Generally, unless otherwise specifically stated, substituent groups usable on molecules herein include any groups, whether substituted or unsubstituted, which do not destroy properties necessary for the photographic utility. Examples of substituents on any of the mentioned groups can include known substituents, such as: halogen, for example, chloro, fluoro, bromo, iodo; alkoxy, particularly those "lower alkyl" (that is, with 1 to 6 carbon atoms, for example, methoxy, ethoxy; substituted or unsubstituted alkyl, particularly lower alkyl (for example, methyl, trifluoromethyl); thioalkyl (for example, methylthio or ethylthio), particularly either of those with 1 to 6 carbon atoms; substituted and unsubstituted aryl, particularly those having from 6 to 20 carbon atoms (for example, phenyl); and substituted or unsubstituted heteroaryl, particularly those having a 5 or 6-membered ring containing 1 to 3 heteroatoms selected from N, O, or S (for example, pyridyl, thiényl, furyl, pyrrolyl); acid or acid salt groups such as any of those described below; and others known in the art. Alkyl substituents may specifically include "lower alkyl" (that is, having 1-6 carbon atoms), for example, methyl, ethyl, and the like. Further, with regard to any alkyl group or alkylene group, it will be understood that these can be branched or unbranched and include ring structures.

In embodiments of the invention in which the emulsion to be used is predominantly AgCl, the invention can be achieved with dyes that: (a) for the two dyes with one allowed 5-position substituent, it must be aromatic in character; and (b) for the dyes with two allowed 5-position substituents, at least one of them must be aromatic in character.

Examples of inventive and comparative dyes are shown in the following Table B. Note that the adjective "comparative" applies for these dyes only in reference to the AgCl emulsion; these dyes fail to aggregate or sustain the invention on this substrate. The predominant feature of this invention is that it applies to pairs of dyes rather than to single dyes.

TABLE B-continued

| Chromo-<br>phore<br>Class | Illustrative Inventive and Comparative Dyes* |                           | 5'-position<br>substituent | 5'-position<br>substituent | Dye<br>Identifier |
|---------------------------|----------------------------------------------|---------------------------|----------------------------|----------------------------|-------------------|
|                           | Inventive (I) or<br>Comparative<br>(C)       | 5-position<br>substituent |                            |                            |                   |
| 10                        | C (AgCl)                                     |                           |                            |                            |                   |
|                           | I                                            |                           | n.a.                       | 1-pyrrolyl                 | E'1               |
|                           | I                                            |                           | n.a.                       | phenyl                     | E'2               |
|                           | D                                            | I                         | chloro                     | phenyl                     | D1                |
|                           | C                                            | I                         | n.a.                       | n.a.                       | C1                |
|                           | B                                            | I                         | n.a.                       | phenyl                     | B1                |
| 15                        | A                                            | I                         | phenyl                     | phenyl                     | A1                |

\*R<sub>1</sub> and R<sub>2</sub> each represent 3-sulfopropyl unless otherwise indicated.

\*n.a. stands for not applicable - the 5-position of the benzo ring is not available for substitution.

This invention describes the use of the combination of at least two blue sensitizing dyes having specifically different structures in combination with a silver halide emulsion so as to adjust the sensitization maximum of the element. This can afford improved color reproduction while maintaining high photographic sensitivity.

Preferred dye combinations are include, for example:

A. the first dye is of the structure:



and the second dye is of the structure:



B. the first dye is of the structure:



and the second dye is of the structure:



TABLE B

Illustrative Inventive and Comparative Dyes\*

| Chromo-<br>phore<br>Class | Inventive (I) or<br>Comparative<br>(C) | 5-position<br>substituent    | 5'-position<br>substituent | Dye<br>Identifier |
|---------------------------|----------------------------------------|------------------------------|----------------------------|-------------------|
| F                         | I                                      | chloro                       | phenyl                     | F1                |
|                           | I                                      | chloro                       | 1-pyrrolyl                 | F2                |
|                           | I (AgBr) or<br>C (AgCl)                | chloro                       | chloro                     | F3                |
|                           | I                                      | phenyl                       | phenyl                     | F4                |
|                           | I                                      | phenylcarbamoyl              | phenyl                     | F5                |
|                           | I                                      | phenylcarboxamido            | phenyl                     | F6                |
|                           | I                                      | phenyl                       | CO <sub>2</sub> Me         | F7                |
|                           | I                                      | fluorophenyl-<br>carboxamido | chloro                     | F8                |
|                           | C                                      | 1-pyrrolyl                   | CF <sub>3</sub>            | F9                |
|                           | C                                      | phenyl                       | CF <sub>3</sub>            | F10               |
| E                         | I                                      | phenyl                       | n.a.**                     | E1                |
|                           | I                                      | 2-thienyl                    | n.a.                       | E2                |
|                           | I                                      | 1-pyrrolyl                   | n.a.                       | E3                |
|                           | I                                      | 2-furyl                      | n.a.                       | E6                |
|                           | I (AgBr) or<br>C (AgCl)                | chloro                       | n.a.                       | E4                |
|                           | I (AgBr) or                            | methoxy                      | n.a.                       | E5                |

**9**

C. the first dye is of the structure:

**10**

F. the first dye is of the structure:



and the second dye is of the structure:



D. the first dye is of the structure:



and the second dye is of the structure:



E. the first dye is of the structure:



and the second dye is of the structure:



10 and the second dye is of the structure:



20 G. the first dye is of the structure:



30 and the second dye is of the structure:



40 H. the first dye is of the structure:



50 and the second dye is of the structure:



60 wherein Z<sub>1</sub>, Z<sub>2</sub> and Z'' are independently a hydrogen or halogen atom or a substituted or unsubstituted alkyl, substituted or unsubstituted alkoxy, substituted or unsubstituted aromatic, substituted or unsubstituted alkoxy carbonyl and substituted or unsubstituted heterocyclic group; and R<sub>1</sub> and R<sub>2</sub>, are independently substituted or unsubstituted alkyl, substituted or unsubstituted alkenyl or substituted or unsubstituted aryl.

Particularly preferred blue dyes for use in this invention are of structures I and II defined below.



Dye I

wherein:

Z1 is phenyl, pyrrolyl, furanyl, thieryl, alkoxycarbonyl or a fused benzene ring;

Z2 is phenyl, pyrrolyl, furanyl, thieryl, alkoxycarbonyl or halogen, R1 and R2 are acid substituted alkyl groups; and

A+ is a counterion,



Dye II

wherein

X is O or S,

Y1 is pyrrolyl, furanyl, thieryl, alkoxycarbonyl or phenyl;

Y2 is a 4,5-benzo substituent when X is O and a phenylcarbamoyl or a phenylcarboxamido substituent when X is S;

R3 and R4 are acid substituted alkyl groups; and

B+ is a counterion.

In the above formulae, A+ and B+ are counterions required to balance the net charge of the dye. Any positively charged counterion can be utilized. Common counterions that can be used include sodium, potassium, triethylammonium (TEA+), tetramethylguanidinium (TMG+), diisopropylammonium (DIPA+), and tetrabutylammonium (TBA+).

These dyes USED in accordance with this invention can be synthesized by those skilled in the art according to the procedures described herein or IN F. M. Hamer, *The Cynine Dyes and Related Compounds* (Interscience Publishers, New York, 1964).

Illustrative preferred dyes are given in Table C

TABLE C



| Dye ID | Z             | Z'             | W |
|--------|---------------|----------------|---|
| F2     | 5-Cl          | 5-(1-Pyrrolyl) | S |
| F3     | 5-Cl          | 5-Cl           | S |
| F4     | 5-Ph          | 5-Ph           | S |
| D1     | 5-Ph          | 5-Cl           | O |
| E4     | 5-Cl          | 4,5-Benzo      | O |
| E1     | 5-Ph          | 4,5-Benzo      | O |
| E2     | 5-(2-Thienyl) | 4,5-Benzo      | O |
| F1     | 5-Phenyl      | 5-Cl           | S |
| E6     | 5-(2-Furanyl) | 4,5-Benzo      | O |

TABLE C-continued

|    |  |
|----|--|
| 5  |  |
| 10 |  |
| 15 |  |
| 20 |  |
| 25 |  |
| 30 |  |
| 35 |  |
| 40 |  |
| 45 |  |
| 50 |  |

The photographic element of the invention comprises a blue sensitive emulsion layer which has been chemically sensitized with a gold(I) compound of formula (Ia) or (Ib):



wherein

L is a mesoionic compound;

X is an anion; and

L1 is a Lewis donor ligand.

The compounds may be soluble in any of a variety of solvents, including water or organic solvents such as acetone or methanol, but the most preferred compounds are water soluble. The term water soluble herein means that the gold(I) compound dissolves in water at the concentration of at least 10-5 mole per liter of water at a temperature of 20° C. at normal pressure.

The mesoionic compound L herein is any such compound that can be coordinated with gold(I) ions to form a gold(I) compound that is water soluble and enables the described chemical sensitization of a photographic silver halide composition. The mesoionic compound is preferably represented by the formula:



wherein the circle with the + sign on the heterocyclic ring symbolizes six delocalized  $\pi$  electrons associated with a partial positive charge on the heterocyclic ring. The a, b, c, d, and e represent the unsubstituted or substituted atoms necessary to complete the mesoionic compound, for example the carbon and nitrogen atoms necessary to complete mesoionic triazolium or tetrazolium 5-member heterocyclic ring. The members of the heterocyclic ring (a, b, c, d, and e) may be CR5 or NR5' groups or chalcogen atoms. The minus sign indicates two additional electrons on the exocyclic group f which are conjugated with the six  $\pi$  electrons on the heterocyclic ring. It is understood that there is extensive delocalization and that the charges indicated are only partial charges. The exocyclic group f may be S, Se, or NR5''. The groups R5, R5' and R5'' may be hydrogen atoms, substituted or unsubstituted alkyl, aryl, or heterocyclic groups, or R5,

$R_5'$  and  $R_5''$  may link together by bonding to form another ring. (Note: Structural representations for mesoionic compounds L which are different from that given above appear elsewhere in the literature, but here the conventions followed are those described by Ollis and Ramsden in *Advances in Heterocyclic Chemistry*, Vol. 19, Academic Press, London (1976). It is through the exocyclic group f that the mesoionic compound coordinates to gold(I) in the compounds used in the present invention. The exocyclic group f should not be O for the present invention since oxygen ligands are not known to form stable compounds with gold(I).

Examples of the gold(I) compounds of the invention are given in the table below. In the structural representations of the gold(I) compounds, the partial charges on the mesoionic ligands are dropped to avoid confusion with the overall charge of the complex ion. The rings symbolizing six delocalized  $\pi$  electrons on the heterocyclic moieties are retained, but will be understood not to imply aromaticity.



wherein  $R_6$ ,  $R_7$ , and  $R_8$  are independently a substituted or unsubstituted alkyl group, a substituted or unsubstituted alkenyl group, an amino group, a substituted or unsubstituted aryl group, and  $X^-$  is a halogen or  $BF_4^-$  anion. Preferred compounds are listed in the following table:

| Compound No. | $R_6$           | $R_7$                              | $R_8$           | $X^-$                        |
|--------------|-----------------|------------------------------------|-----------------|------------------------------|
| 1            | CH <sub>3</sub> | CH <sub>3</sub>                    | CH <sub>3</sub> | BF <sub>4</sub> <sup>-</sup> |
| 2            | CH <sub>3</sub> | CH <sub>3</sub>                    | CH <sub>3</sub> | I <sup>-</sup>               |
| 3            | CH <sub>3</sub> | CH <sub>3</sub>                    | CH <sub>3</sub> | Br <sup>-</sup>              |
| 4            | CH <sub>3</sub> | CH <sub>3</sub>                    | CH <sub>3</sub> | Cl <sup>-</sup>              |
| 5            | CH <sub>3</sub> | CH <sub>2</sub> CH=CH <sub>2</sub> | CH <sub>3</sub> | BF <sub>4</sub> <sup>-</sup> |
| 6            | CH <sub>3</sub> | CH <sub>2</sub> CHOCH <sub>3</sub> | CH <sub>3</sub> | BF <sub>4</sub> <sup>-</sup> |
| 7            | CH <sub>3</sub> | NH <sub>2</sub>                    | CH <sub>3</sub> | BF <sub>4</sub> <sup>-</sup> |
| 8            | CH <sub>3</sub> | C <sub>4</sub> H <sub>9</sub>      | CH <sub>3</sub> | BF <sub>4</sub> <sup>-</sup> |
| 9            | CH <sub>3</sub> | C <sub>6</sub> H <sub>11</sub>     | CH <sub>3</sub> | BF <sub>4</sub> <sup>-</sup> |
| 10           | CH <sub>3</sub> | C <sub>6</sub> H <sub>5</sub>      | CH <sub>3</sub> | BF <sub>4</sub> <sup>-</sup> |



wherein  $R_6$ ,  $R_7$  and  $X^-$  are as defined above. Preferred compounds are given in the following table:

| Compound No. | $R_6$                         | $R_7$                         | $X^-$                        |
|--------------|-------------------------------|-------------------------------|------------------------------|
| 11           | C <sub>6</sub> H <sub>5</sub> | C <sub>6</sub> H <sub>5</sub> | BF <sub>4</sub> <sup>-</sup> |

wherein  $R_6$ ,  $R_7$ ,  $R_8$ , and  $R_9$  are independently a substituted or unsubstituted alkyl group, a substituted or unsubstituted alkenyl group, an amino group, a substituted or unsubstituted aryl group, and  $X^-$  is a halogen or  $BF_4^-$  anion. Preferred compounds are listed in the following table:

| Compound No. | $R_6$           | $R_7$                              | $R_8$           | $R_9$           | $X^-$                        |
|--------------|-----------------|------------------------------------|-----------------|-----------------|------------------------------|
| 12           | CH <sub>3</sub> | CH <sub>3</sub>                    | CH <sub>3</sub> | CH <sub>3</sub> | Cl <sup>-</sup>              |
| 13           | CH <sub>3</sub> | CH <sub>3</sub>                    | CH <sub>3</sub> | CH <sub>3</sub> | BF <sub>4</sub> <sup>-</sup> |
| 14           | CH <sub>3</sub> | CH <sub>2</sub> CH=CH <sub>2</sub> | CH <sub>3</sub> | CH <sub>3</sub> | BF <sub>4</sub> <sup>-</sup> |

These gold(I) compounds are advantageous over certain other gold compounds containing sulfur known in the art such as trisodium aurous dithiosulfate because the compounds do not contain any labile S atoms, thus allowing independent choice and amount of S sensitizer, which is not possible with trisodium aurous dithiosulfate. The flexibility in choice and amount of sulfur sensitizer to be used in photographic emulsion is necessary in some cases to achieve proper gradation, reduced sensitivity to red light, and other sensitometric properties. The gold (I) compounds utilized in the present invention have a lower dissociation constant than prior art gold (I) compounds and consequently have better solution stability. Alkyl or aryl thiolates, for example, have a propensity to form polymeric gold(I) compounds with a 1:1 thiolate to gold formula. The compounds of this invention contain discrete gold(I) complexes possessing two ligands. Consequently, the compounds have solubility properties which are convenient for dispersion in the emulsion without requiring that a sulfonic acid or other solubilizing group be attached to the ligand. The compounds of the present invention also are advantageous over prior art gold (I) compounds in that they are very convenient and does not involve potentially explosive material.

The mesoionic compounds L used as starting materials to form the compounds with gold(I) may be made by methods described by Altland, Dedio and McSweeney, U.S. Pat. No. 4,378,424 (1983) or by methods described in the review article by Ollis and Ramsden cited above and references given therein. Synthesis of the gold(I) compounds can be effected by various techniques known to the art. One convenient method comprises reacting a gold(I) precursor compound with an appropriate amount of the mesoionic compound. In the ensuing reaction, which generally takes place with a few minutes at room temperature (about 20° C.) or slightly above, the ligands of the gold(I) precursor compound are displaced by the mesoionic compounds, which have a higher affinity for gold(I). The product may then be isolated and purified by crystallization techniques.

The various substituent groups on the mesoionic compound modify the solubility of the final product gold(I)

compound. The most desired gold(I) compounds are those which are soluble in water and which may be made in water. Those which are soluble in organic solvents such as acetone can still be used to sensitize aqueous emulsions, and can be used to sensitize emulsions in non-aqueous media. The gold compounds are described in more detail in U.S. Pat. No. 5,049,485, the entire disclosure of which is incorporated herein by reference.

Disulfide compound used in the photographic element of this invention is preferably a compound represented by formula (II):



wherein:

X' is independently —O—, —NH— or —NR—, where R is an alkyl group, a fluoroalkyl group, an aryl group or a sulfonyl group;

m and r are independently 0, 1 or 2, with the proviso that m and r are not both 0;

M is —H or a cationic species;

Ar is an aromatic group;

p is 0 or 1; and

L² is a linking group, where p is 1.

Ar is an aromatic group either of a single ring or a condensed ring, preferably having 6 to 10 carbon atoms and more preferably having 6 carbon atoms. Examples of suitable aromatic groups include naphthyl and phenyl. Ar may be further substituted or may be unsubstituted, more preferably Ar is unsubstituted. Examples of suitable substituents include alkyl groups (for example, methyl, ethyl, hexyl), fluoroalkyl groups (for example, trifluoromethyl), alkoxy groups (for example, methoxy, ethoxy, octyloxy), aryl groups (for example, phenyl, naphthyl, tolyl), hydroxyl groups, halogen atoms, aryloxy groups (for example, phenoxy), alkylthio groups (for example, methylthio, butylthio), arylthio groups (for example, phenylthio), acyl groups (for example, acetyl, propionyl, butyryl, valeryl), sulfonyl groups (for example, methylsulfonyl, phenylsulfonyl), acylamino groups, sulfonylamino groups, acyloxy groups (for example, acetoxy, benzoxy), carboxyl groups, cyano groups, sulfo groups, and amino groups. Preferred are simple alkyl groups and acylamino groups.

X' is independently an —O—, —NH— or —NR—. Most preferably X is —NH—. If X is —NR—, R is a substituent which does not interfere with the intended function of the disulfide compound in the photographic emulsion and which maintains the water solubility of the compound. Examples of suitable substituents include alkyl groups (for example, methyl, ethyl, hexyl), fluoroalkyl groups (for example, trifluoromethyl), aryl groups (for example, phenyl, naphthyl, tolyl), sulfonyl groups (for example, methylsulfonyl, phenylsulfonyl). Preferred are simple alkyl groups and simple fluoroalkyl groups.

r and m are independently 0, 1 or 2. Therefore, included are those compounds in which only one of the aromatic

groups is substituted. Preferably m and r are both 1. X' is independently in any position in the aromatic nucleus relative to the sulfur. More preferably, the molecule is symmetrical and preferably X' is either in the para or ortho position.

L² is a linking group. p is 0 or 1. Preferably L² is an unsubstituted alkylene group and is usually —(CH<sub>2</sub>)<sub>n</sub>— where n ranges from zero to 11 and is preferably 1 to 3. Other examples of L' are given below,



M is either a hydrogen atom or a cationic species if the carboxyl group is in its ionized form. The cationic species may be a metal ion or an organic ion. Examples of organic cations include ammonium ions (for example, ammonium, tetramethylammonium, tetrabutylammonium), phosphonium ions (for example, tetraphenylphosphonium), and guanidyl groups. Preferably M is hydrogen or an alkali metal cation, with a sodium or potassium ion being most preferred.

Examples of the disulfide compounds of this invention are shown below. Compounds I-A through I-H are preferred with Compounds I-D and I-E being most preferred.





19

-continued



The solubilized disulfides of this invention are easily prepared using readily available starting materials. Most of the solubilized disulfides can be obtained by reacting aminophenyl disulfide or hydroxyphenyl disulfide with the appropriate cyclic anhydride followed by conversion of the free diacid to its anionic form using materials such as sodium bicarbonate. Other solubilized disulfides could be obtained by reacting aminophenyl disulfide or hydroxyphenyl disulfide with the mono chloride of a dicarboxylic acid mono ester, followed by hydrolysis of the ester to the carboxylic acid. A discussion of these disulfide compounds can be found in U.S. Pat. No. 5,418,127, the entire disclosure of which is incorporated herein by reference.

The emulsion layer of the photographic element of the invention can comprise any one or more of the light sensitive layers of the photographic element. The photographic elements made in accordance with the present invention can be black and white elements, single color elements or multi-color elements. Multicolor elements contain dye image-forming units sensitive to each of the three primary regions of the spectrum. Each unit can be comprised of a single emulsion layer or of multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

A typical multicolor photographic element comprises a support bearing a cyan dye image-forming unit comprised of at least one red-sensitive silver halide emulsion layer having associated therewith at least one cyan dye-forming coupler, a magenta dye image-forming unit comprising at least one green-sensitive silver halide emulsion layer having associated therewith at least one magenta dye-forming coupler, and a yellow dye image-forming unit comprising at least one blue-sensitive silver halide emulsion layer having associated therewith at least one yellow dye-forming coupler. The element can contain additional layers, such as filter layers, interlayers, overcoat layers, subbing layers, antihalation layers and the like. All of these can be coated on a support which can be transparent or reflective (for example, a paper support).

20

Photographic elements of the present invention may also usefully include a magnetic recording material as described in *Research Disclosure*, Item 34390, November 1992, or a transparent magnetic recording layer such as a layer containing magnetic particles on the underside of a transparent support as in U.S. Pat. No. 4,279,945 and U.S. Pat. No. 4,302,523. The element typically will have a total thickness (excluding the support) of from 5 to 30 microns. While the order of the color sensitive layers can be varied, they will normally be red-sensitive, green-sensitive and blue-sensitive, in that order on a transparent support, (that is, blue sensitive furthest from the support) and the reverse order on a reflective support being typical.

The present invention also contemplates the use of photographic elements of the present invention in what are often referred to as single use cameras (or "film with lens" units). These cameras are sold with film preloaded in them and the entire camera is returned to a processor with the exposed film remaining inside the camera. Such cameras may have glass or plastic lenses through which the photographic element is exposed.

In the following discussion of suitable materials for use in elements of this invention, reference will be made to *Research Disclosure*, September 1996, Number 389, Item 38957, which will be identified hereafter by the term "Research Disclosure I." The Sections hereafter referred to are Sections of the Research Disclosure I unless otherwise indicated. All Research Disclosures referenced are published by Kenneth Mason Publications, Ltd., Dudley Annex, 12a North Street, Emsworth, Hampshire P010 7DQ, ENGLAND. The foregoing references and all other references cited in this application, are incorporated herein by reference.

The silver halide emulsions employed in the photographic elements of the present invention may be negative-working, such as surface-sensitive emulsions or unfogged internal latent image forming emulsions, or positive working emulsions of the internal latent image forming type (that are fogged during processing). Suitable emulsions and their preparation as well as methods of chemical and spectral sensitization are described in Sections I through V. Color materials and development modifiers are described in Sections V through XX. Vehicles which can be used in the photographic elements are described in Section II, and various additives such as brighteners, antifoggants, stabilizers, light absorbing and scattering materials, hardeners, coating aids, plasticizers, lubricants and matting agents are described, for example, in Sections VI through XIII. Manufacturing methods are described in all of the sections, layer arrangements particularly in Section XI, exposure alternatives in Section XVI, and processing methods and agents in Sections XIX and XX.

With negative working silver halide a negative image can be formed. Optionally a positive (or reversal) image can be formed although a negative image is typically first formed.

The photographic elements of the present invention may also use colored couplers (e.g. to adjust levels of interlayer correction) and masking couplers such as those described in EP 213 490; Japanese Published Application 58-172,647; U.S. Pat. No. 2,983,608; German Application DE 2,706,117C; U.K. Patent 1,530,272; Japanese Application A-1 13935; U.S. Pat. No. 4,070,191 and German Application DE 2,643,965. The masking couplers may be shifted or blocked.

The photographic elements may also contain materials that accelerate or otherwise modify the processing steps of bleaching or fixing to improve the quality of the image. Bleach accelerators described in EP 193 389; EP 301 477;

U.S. Pat. No. 4,163,669; U.S. Pat. No. 4,865,956; and U.S. Pat. No. 4,923,784 are particularly useful. Also contemplated is the use of nucleating agents, development accelerators or their precursors (UK Patent 2,097,140; U.K. Patent 2,131,188); development inhibitors and their precursors (U.S. Pat. No. 5,460,932; U.S. Pat. No. 5,478,711); electron transfer agents (U.S. Pat. No. 4,859,578; U.S. Pat. No. 4,912,025); antifogging and anti color-mixing agents such as derivatives of hydroquinones, aminophenols, amines, gallic acid; catechol; ascorbic acid; hydrazides; sulfonamidophenols; and non color-forming couplers.

The elements may also contain filter dye layers comprising colloidal silver sol or yellow and/or magenta filter dyes and/or antihalation dyes (particularly in an undercoat beneath all light sensitive layers or in the side of the support opposite that on which all light sensitive layers are located) either as oil-in-water dispersions, latex dispersions or as solid particle dispersions. Additionally, they may be used with "smearing" couplers (e.g. as described in U.S. Pat. No. 4,366,237; EP 096 570; U.S. Pat. No. 4,420,556; and U.S. Pat. No. 4,543,323.) Also, the couplers may be blocked or coated in protected form as described, for example, in Japanese Application 61/258,249 or U.S. Pat. No. 5,019,492.

The photographic elements may further contain other image-modifying compounds such as "Development Inhibitor-Releasing" compounds (DIR's). Useful additional DIR's for elements of the present invention, are known in the art and examples are described in U.S. Pat. Nos. 3,137,578; 3,148,022; 3,148,062; 3,227,554; 3,384,657; 3,379,529; 3,615,506; 3,617,291; 3,620,746; 3,701,783; 3,733,201; 4,049,455; 4,095,984; 4,126,459; 4,149,886; 4,150,228; 4,211,562; 4,248,962; 4,259,437; 4,362,878; 4,409,323; 4,477,563; 4,782,012; 4,962,018; 4,500,634; 4,579,816; 4,607,004; 4,618,571; 4,678,739; 4,746,600; 4,746,601; 4,791,049; 4,857,447; 4,865,959; 4,880,342; 4,886,736; 4,937,179; 4,946,767; 4,948,716; 4,952,485; 4,956,269; 4,959,299; 4,966,835; 4,985,336 as well as in patent publications GB 1,560,240; GB 2,007,662; GB 2,032,914; GB 2,099,167; DE 2,842,063, DE 2,937,127; DE 3,636,824; DE 3,644,416 as well as the following European Patent Publications: 272,573; 335,319; 336,41 1; 346,899; 362,870; 365,252; 365,346; 373,382; 376,212; 377,463; 378,236; 384,670; 396,486; 401,612; 401,613.

DIR compounds are also disclosed in "Developer-Inhibitor-Releasing (DIR) Couplers for Color Photography," C. R. Barr, J. R. Thirtle and P. W. Vittum in *Photographic Science and Engineering*, Vol. 13, p. 174 (1969), incorporated herein by reference.

It is also contemplated that the concepts of the present invention may be employed to obtain reflection color prints as described in *Research Disclosure*, November 1979, Item 18716, available from Kenneth Mason Publications, Ltd, Dudley Annex, 12a North Street, Emsworth, Hampshire P0101 7DQ, England, incorporated herein by reference. The emulsions and materials to form elements of the present invention, may be coated on pH adjusted support as described in U.S. Pat. No. 4,917,994; with epoxy solvents (EP 0 164 961); with additional stabilizers (as described, for example, in U.S. Pat. No. 4,346,165; U.S. Pat. No. 4,540,653 and U.S. Pat. No. 4,906,559); with ballasted chelating agents such as those in U.S. Pat. No. 4,994,359 to reduce sensitivity to polyvalent cations such as calcium; and with stain reducing compounds such as described in U.S. Pat. No. 5,068,171 and U.S. Pat. No. 5,096,805. Other compounds which may be useful in the elements of the invention are disclosed in Japanese Published Applications 83-09,959;

83-62,586; 90-072,629; 90-072,630; 90-072,632; 90-072,633; 90-072,634; 90-077,822; 90-078,229; 90-078,230; 90-079,336; 90-079,338; 90-079,690; 90-079,691; 90-080,487; 90-080,489; 90-080,490; 90-080,491; 90-080,492; 90-080,494; 90-085,928; 90-086,669; 90-086,670; 90-087,361; 90-087,362; 90-087,363; 90-087,364; 90-088,096; 90-088,097; 90-093,662; 90-093,663; 90-093,664; 90-093,665; 90-093,666; 90-093,668; 90-094,055; 90-094,056; 90-101,937; 90-103,409; 90-151,577.

10 The silver halide used in the photographic elements may be silver iodobromide, silver bromide, silver chloride, silver chlorobromide, silver chloroiodobromide, and the like.

15 The type of silver halide grains preferably include polymorphic, cubic, and octahedral. The grain size of the silver halide may have any distribution known to be useful in photographic compositions, and may be either polydispersed or monodispersed.

Tabular grain silver halide emulsions may also be used. Tabular grains are those with two parallel major faces each clearly larger than any remaining grain face and tabular grain emulsions are those in which the tabular grains account for at least 30 percent, more typically at least 50 percent, preferably >70 percent and optimally >90 percent of total grain projected area. The tabular grains can account for 25 substantially all (>97 percent) of total grain projected area. The tabular grain emulsions can be high aspect ratio tabular grain emulsions—i.e., ECD/t>8, where ECD is the diameter of a circle having an area equal to grain projected area and t is tabular grain thickness; intermediate aspect ratio tabular grain emulsions—i.e., ECD/t=5 to 8; or low aspect ratio tabular grain emulsions—i.e., ECD/t=2 to 5. The emulsions typically exhibit high tabularity (T), where T (i.e., ECD/t<sup>2</sup>)>25 and ECD and t are both measured in micrometers ( $\mu\text{m}$ ). The tabular grains can be of any thickness compatible with achieving an aim average aspect ratio and/or average tabularity of the tabular grain emulsion. Preferably the tabular grains satisfying projected area requirements are those having thicknesses of <0.3  $\mu\text{m}$ , thin (<0.2  $\mu\text{m}$ ) tabular grains being specifically preferred and ultrathin (<0.07  $\mu\text{m}$ ) tabular grains being contemplated for maximum tabular grain performance enhancements. When the native blue absorption of iodothalide tabular grains are relied upon for blue speed, thicker tabular grains, typically up to 0.5  $\mu\text{m}$  in thickness, are contemplated.

45 High iodide tabular grain emulsions are illustrated by House U.S. Pat. No. 4,490,458, Maskasky U.S. Pat. No. 4,459,353 and Yagi et al EPO 0 410 410.

Tabular grains formed of silver halide(s) that form a face centered cubic (rock salt type) crystal lattice structure can 50 have either {100} or {111} major faces. Emulsions containing {111} major face tabular grains, including those with controlled grain dispersities, halide distributions, twin plane spacing, edge structures and grain dislocations as well as adsorbed {111} grain face stabilizers, are illustrated in those 55 references cited in *Research Disclosure I*, Section I.B.(3) (page 503).

The silver halide grains to be used in the invention may 60 be prepared according to methods known in the art, such as those described in *Research Disclosure I* and James, *The Theory of the Photographic Process*. These include methods such as ammoniacal emulsion making, neutral or acidic emulsion making, and others known in the art. These methods generally involve mixing a water soluble silver salt with a water soluble halide salt in the presence of a protective colloid, and controlling the temperature, pAg, pH values, etc, at suitable values during formation of the silver halide 65 by precipitation.

In the course of grain precipitation one or more dopants (grain occlusions other than silver and halide) can be introduced to modify grain properties. For example, any of the various conventional dopants disclosed in *Research Disclosure*, Item 38957, Section I. Emulsion grains and their preparation, sub-section G. Grain modifying conditions and adjustments, paragraphs (3), (4) and (5), can be present in the emulsions of the invention. In addition it is specifically contemplated to dope the grains with transition metal hexacoordination complexes containing one or more organic ligands, as taught by Olm et al U.S. Pat. No. 5,360,712, the disclosure of which is here incorporated by reference.

It is specifically contemplated to incorporate in the face centered cubic crystal lattice of the grains a dopant capable of increasing imaging speed by forming a shallow electron trap (hereinafter also referred to as a SET) as discussed in *Research Disclosure* Item 36736 published November 1994, here incorporated by reference.

The SET dopants are effective at any location within the grains. Generally better results are obtained when the SET dopant is incorporated in the exterior 50 percent of the grain, based on silver. An optimum grain region for SET incorporation is that formed by silver ranging from 50 to 85 percent of total silver forming the grains. The SET can be introduced all at once or run into the reaction vessel over a period of time while grain precipitation is continuing. Generally SET forming dopants are contemplated to be incorporated in concentrations of at least  $1 \times 10^{-7}$  mole per silver mole up to their solubility limit, typically up to about  $5 \times 10^{-4}$  mole per silver mole.

SET dopants are known to be effective to reduce reciprocity failure. In particular the use of iridium hexacoordination complexes or  $\text{Ir}^{+4}$  complexes as SET dopants is advantageous.

Iridium dopants that are ineffective to provide shallow electron traps (non-SET dopants) can also be incorporated into the grains of the silver halide grain emulsions to reduce reciprocity failure. To be effective for reciprocity improvement the Ir can be present at any location within the grain structure. A preferred location within the grain structure for Ir dopants to produce reciprocity improvement is in the region of the grains formed after the first 60 percent and before the final 1 percent (most preferably before the final 3 percent) of total silver forming the grains has been precipitated. The dopant can be introduced all at once or run into the reaction vessel over a period of time while grain precipitation is continuing. Generally reciprocity improving non-SET Ir dopants are contemplated to be incorporated at their lowest effective concentrations.

The contrast of the photographic element can be further increased by doping the grains with a hexacoordination complex containing a nitrosyl or thionitrosyl ligand (NZ dopants) as disclosed in McDugle et al U.S. Pat. No. 4,933,272, the disclosure of which is here incorporated by reference.

The contrast increasing dopants can be incorporated in the grain structure at any convenient location. However, if the NZ dopant is present at the surface of the grain, it can reduce the sensitivity of the grains. It is therefore preferred that the NZ dopants be located in the grain so that they are separated from the grain surface by at least 1 percent (most preferably at least 3 percent) of the total silver precipitated in forming the silver iodochloride grains. Preferred contrast enhancing concentrations of the NZ dopants range from  $1 \times 10^{-11}$  to  $4 \times 10^{-8}$  mole per silver mole, with specifically preferred concentrations being in the range from  $10^{-10}$  to  $10^{-8}$  mole per silver mole.

Although generally preferred concentration ranges for the various SET, non-SET Ir and NZ dopants have been set out above, it is recognized that specific optimum concentration ranges within these general ranges can be identified for specific applications by routine testing. It is specifically contemplated to employ the SET, non-SET Ir and NZ dopants singly or in combination. For example, grains containing a combination of an SET dopant and a non-SET Ir dopant are specifically contemplated. Similarly SET and NZ dopants can be employed in combination. Also NZ and Ir dopants that are not SET dopants can be employed in combination. Finally, the combination of a non-SET Ir dopant with a SET dopant and an NZ dopant. For this latter three-way combination of dopants it is generally most convenient in terms of precipitation to incorporate the NZ dopant first, followed by the SET dopant, with the non-SET Ir dopant incorporated last.

The photographic elements of the present invention, as is typical, provide the silver halide in the form of an emulsion. Photographic emulsions generally include a vehicle for coating the emulsion as a layer of a photographic element. Useful vehicles include both naturally occurring substances such as proteins, protein derivatives, cellulose derivatives (e.g., cellulose esters), gelatin (e.g., alkali-treated gelatin such as cattle bone or hide gelatin, or acid treated gelatin such as pigskin gelatin), deionized gelatin, gelatin derivatives (e.g., acetylated gelatin, phthalated gelatin, and the like), and others as described in *Research Disclosure* I. Also useful as vehicles or vehicle extenders are hydrophilic water-permeable colloids. These include synthetic polymeric peptizers, carriers, and/or binders such as poly(vinyl alcohol), poly(vinyl lactams), acrylamide polymers, polyvinyl acetals, polymers of alkyl and sulfoalkyl acrylates and methacrylates, hydrolyzed polyvinyl acetates, polyamides, polyvinyl pyridine, methacrylamide copolymers, and the like, as described in *Research Disclosure* I. The vehicle can be present in the emulsion in any amount useful in photographic emulsions. The emulsion can also include any of the addenda known to be useful in photographic emulsions.

The silver halide to be used in the invention may be advantageously subjected to chemical sensitization. Compounds and techniques useful for chemical sensitization of silver halide are known in the art and described in *Research Disclosure* I and the references cited therein. Compounds useful as chemical sensitizers, include, for example, active gelatin, sulfur, selenium, tellurium, gold, platinum, palladium, iridium, osmium, rhenium, phosphorous, or combinations thereof. Chemical sensitization is generally carried out at pAg levels of from 5 to 10, pH levels of from 2 to 8, and temperatures of from 30 to 80° C., as described in *Research Disclosure* I, Section IV (pages 510-511) and the references cited therein.

The silver halide may be sensitized by sensitizing dyes by any method known in the art, such as described in *Research Disclosure* I. The dye may be added to an emulsion of the silver halide grains and a hydrophilic colloid at any time prior to (e.g., during or after chemical sensitization) or simultaneous with the coating of the emulsion on a photographic element. The dyes may, for example, be added as a solution in water or an alcohol. The dye/silver halide emulsion may be mixed with a dispersion of color image-forming coupler immediately before coating or in advance of coating (for example, 2 hours).

Photographic elements of the present invention are preferably imagewise exposed using any of the known techniques, including those described in *Research Disclosure* I, section XVI. This typically involves exposure to light

in the visible region of the spectrum, and typically such exposure is of a live image through a lens, although exposure can also be exposure to a stored image (such as a computer stored image) by means of light emitting devices (such as light emitting diodes, CRT and the like).

Photographic elements comprising the composition of the invention can be processed in any of a number of well-known photographic processes utilizing any of a number of well-known processing compositions, described, for example, in *Research Disclosure I*, or in T. H. James, editor, *The Theory of the Photographic Process*, 4th Edition, Macmillan, New York, 1977. In the case of processing a negative working element, the element is treated with a color developer (that is one which will form the colored image dyes with the color couplers), and then with an oxidizer and a solvent to remove silver and silver halide. In the case of processing a reversal color element, the element is first treated with a black and white developer (that is, a developer which does not form colored dyes with the coupler compounds) followed by a treatment to fog silver halide (usually chemical fogging or light fogging), followed by treatment with a color developer. Preferred color developing agents are p-phenylenediamines. Especially preferred are: 4-amino N,N-diethylaniline hydrochloride, 4-amino-3-methyl-N,N-diethylaniline hydrochloride, 4-amino-3-methyl-N-ethyl-N-(methanesulfonamido) ethylaniline sesquisulfate hydrate, 4-amino-3-methyl-N-ethyl-N-(β-hydroxyethyl)aniline sulfate, 4-amino-3-β-(methanesulfonamido)ethyl-N,N-diethylaniline hydrochloride and 4-amino-N-ethyl-N-(2-methoxyethyl)-m-toluidine di-p-toluene sulfonic acid.

Dye images can be formed or amplified by processes which employ in combination with a dye-image-generating reducing agent an inert transition metal-ion complex oxidizing agent, as illustrated by Bissonette U.S. Pat. Nos. 3,748,138, 3,826,652, 3,862,842 and 3,989,526 and Travis U.S. Pat. No. 3,765,891, and/or a peroxide oxidizing agent as illustrated by Matejec U.S. Pat. No. 3,674,490, *Research Disclosure*, Vol. 116, December, 1973, Item 11660, and Bissonette *Research Disclosure*, Vol. 148, August, 1976, Items 14836, 14846 and 14847. The photographic elements can be particularly adapted to form dye images by such processes as illustrated by Dunn et al U.S. Pat. No. 3,822,129, Bissonette U.S. Pat. Nos. 3,834,907 and 3,902,905, Bissonette et al U.S. Pat. No. 3,847,619, Mowrey U.S. Pat. No. 3,904,413, Hirai et al U.S. Pat. No. 4,880,725, Iwano U.S. Pat. No. 4,954,425, Marsden et al U.S. Pat. No. 4,983,504, Evans et al U.S. Pat. No. 5,246,822, Twist U.S. Pat. No. 5,324,624, Fyson EPO 0 487 616, Tannahill et al WO 90/13059, Marsden et al WO 90/13061, Grimsey et al WO 91/16666, Fyson WO 91/17479, Marsden et al WO 92/01972, Tannahill WO 92/05471, Henson WO 92/07299, Twist WO 93/01524 and WO 93/11460 and Wingender et al German OLS 4,211,460.

Development is followed by bleach-fixing, to remove silver or silver halide, washing and drying.

The following examples illustrate the use of the dye combinations of the invention.

#### EXAMPLE 1

This example demonstrates the use of dye combinations of this invention with a cubic AgCl emulsion.

In this experiment, a pure AgCl emulsion of predominantly cubic morphology was used. The median grain size was 0.39 micron cubic edge length (CEL). The emulsion

was chemically sensitized (finished) by melting the emulsion at 40 degrees C., then adding colloidal aurous sulfide at 0.0177 g per mole of AgCl, and heating the emulsion to 65 degrees C. for 55 minutes prior to chilling the emulsion.

The sensitizing dyes were added by re-melting the emulsion at 40 degrees C., and adding the dyes from methanolic solutions at a concentration of 0.000471 moles per liter to produce a dye-to-silver ratio of  $3.8 \times 10^{-4}$  moles of dye per silver mole. The emulsion was held with stirring for 20 minutes, then chilled with stirring.

The two dyes comprising a particular combination were tested by adding each of them individually to the emulsion, and also by adding them to the emulsion simultaneously from pre-mixed co-solutions in the percentages 75% Dye 1, 25% Dye 2; 50% Dye 1, 50% Dye 2; 25% Dye 1, 75% Dye 2.

The dyed emulsions were coated onto an ESTAR™ support using a coating machine equipped with an extrusion device to deliver the melted emulsion onto the support.

The melt as coated consisted of emulsion, gelatin, water, dye solutions as described above, the surfactant saponin (which is a naturally occurring glycoside), and the hardener 1,1'-(oxybis-(methylenesulfonyl)bis-)ethene (BVSME).

The total "wet" laydown was 157.2 g/m<sup>2</sup> (14.6 mg/ft<sup>2</sup>). After chilling and drying, the resulting single-layer coatings contained 3229 mg/m<sup>2</sup> of silver, 7319 mg/m<sup>2</sup> of gelatin, 122.6 mg/m<sup>2</sup> of BVSME, and 144.8 mg/m<sup>2</sup> of saponin.

A spectrum was obtained of the coated material using a scanning spectrophotometer equipped with an integrating sphere. The coated materials were exposed with a sensitometer equipped with a tungsten light source which is filtered with a collection of Wratten filters designed to approximate exposure through a color film negative. A step tablet was used to provide a D logE curve from which photographic speed at 0.8 density units above Dmin was determined, as is familiar to those skilled in the art.

The exposed strips were developed in the following process at 20 degrees C.

1. KODAK DK-50™ developer for 6 minutes, 0 seconds.
2. KODAK INDICATOR STOP™ stop bath for 15 seconds.
3. KODAK F5™ fix for 5 minutes 0 seconds.
4. Distilled water wash for 10 minutes 0 seconds.

The data from this experiment for a variety of inventive and comparative dye pairs is shown in Table I.

TABLE I

Data Obtained for Pairs of Dyes on AgCl Cubic Emulsion.  
I = inventive. C = comparative.

| Type | Long<br>Dye | Short<br>Dye | ΔE<br>(eV) | Ratio<br>(% long<br>dye) |          | Aggregate<br>Wave-<br>length<br>(nm) | Aggregate<br>Peak<br>Height<br>(% A)* | Speed** |
|------|-------------|--------------|------------|--------------------------|----------|--------------------------------------|---------------------------------------|---------|
|      |             |              |            | 100                      | 465      |                                      |                                       |         |
| C    | F1          | D1           | 0.15       | 75                       | 462      | 56.1                                 | 139                                   | 144     |
|      |             |              |            | 50                       | 459      | 53.0                                 | 135                                   |         |
|      |             |              |            | 25                       | 440      | 48.3                                 | 124                                   |         |
|      |             |              |            | 0                        | 440      | 58.0                                 | 101                                   |         |
|      |             |              |            |                          |          |                                      |                                       |         |
| C    | D1          | C1           | —          | 100                      | 439.2    | 55.2                                 | n.a.***                               | n.a.*** |
|      |             |              |            | 75                       | 438.7    | 51.4                                 | n.a.                                  |         |
|      |             |              |            | 50                       | 438.5    | 43.0                                 | n.a.                                  |         |
|      |             |              |            | 25                       | 437.7    | 29.5                                 | n.a.                                  |         |
|      |             |              |            | 0                        | no peak; | does not                             | aggregate                             |         |

TABLE I-continued

| Data Obtained for Pairs of Dyes on AgCl Cubic Emulsion.<br>I = inventive. C = comparative. |             |              |                    |                          |                                      |                                       |           |
|--------------------------------------------------------------------------------------------|-------------|--------------|--------------------|--------------------------|--------------------------------------|---------------------------------------|-----------|
| Type                                                                                       | Long<br>Dye | Short<br>Dye | $\Delta E$<br>(eV) | Ratio<br>(% long<br>dye) | Aggregate<br>Wave-<br>length<br>(nm) | Aggregate<br>Peak<br>Height<br>(% A)* | Speed**   |
|                                                                                            |             |              |                    |                          |                                      |                                       |           |
| C                                                                                          | C1          | B1           | —                  | 100                      | no peak;                             | does not                              | aggregate |
|                                                                                            |             |              |                    | 75                       | no peak;                             | does not                              | aggregate |
|                                                                                            |             |              |                    | 50                       | 424.1                                | 36.4                                  | n.a.      |
|                                                                                            |             |              |                    | 25                       | 423.1                                | 45.3                                  | n.a.      |
|                                                                                            |             |              |                    | 0                        | 421.0                                | 49.0                                  | n.a.      |
| I                                                                                          | B1          | A1           | 0.09               | 100                      | 421.0                                | 49.0                                  | n.a.      |
|                                                                                            |             |              |                    | 75                       | 418.0                                | 47.9                                  | n.a.      |
|                                                                                            |             |              |                    | 50                       | 412.0                                | 48.1                                  | n.a.      |
|                                                                                            |             |              |                    | 25                       | 409.3                                | 51.4                                  | n.a.      |
|                                                                                            |             |              |                    | 0                        | 408.3                                | 53.8                                  | n.a.      |
| I                                                                                          | F2          | E1           | 0.11               | 100                      | 470                                  | 60.9                                  | 145       |
|                                                                                            |             |              |                    | 75                       | 467                                  | 58.0                                  | 143       |
|                                                                                            |             |              |                    | 50                       | 462                                  | 55.8                                  | 138       |
|                                                                                            |             |              |                    | 25                       | 455                                  | 56.4                                  | 131       |
|                                                                                            |             |              |                    | 0                        | 451                                  | 59.5                                  | 116       |
| I                                                                                          | F2          | E2           | 0.08               | 100                      | 470.4                                | 56.3                                  | 150       |
|                                                                                            |             |              |                    | 75                       | 467.8                                | 55.1                                  | 147       |
|                                                                                            |             |              |                    | 50                       | 464.7                                | 51.1                                  | 133       |
|                                                                                            |             |              |                    | 25                       | 460.9                                | 55.9                                  | 136       |
|                                                                                            |             |              |                    | 0                        | 456.9                                | 56.4                                  | 122       |
| I                                                                                          | F2          | E6           | 0.07               | 100                      | 470.4                                | 56.3                                  | 150       |
|                                                                                            |             |              |                    | 75                       | 467.9                                | 56.0                                  | 139       |
|                                                                                            |             |              |                    | 50                       | 464.9                                | 54.9                                  | 129       |
|                                                                                            |             |              |                    | 25                       | 461.2                                | 52.8                                  | 113       |
|                                                                                            |             |              |                    | 0                        | 457.9                                | 54.4                                  | 97        |
| I                                                                                          | F2          | E3           | 0.09               | 100                      | 470.0                                | 52.3                                  | 137       |
|                                                                                            |             |              |                    | 75                       | 465.5                                | 52.3                                  | 136       |
|                                                                                            |             |              |                    | 50                       | 461.1                                | 52.5                                  | 132       |
|                                                                                            |             |              |                    | 25                       | 457.1                                | 55.4                                  | 126       |
|                                                                                            |             |              |                    | 0                        | 454.3                                | 59.7                                  | 118       |
| I                                                                                          | F1          | E1           | 0.08               | 100                      | 464.7                                | 60.3                                  | 136       |
|                                                                                            |             |              |                    | 75                       | 462.4                                | 59.5                                  | 133       |
|                                                                                            |             |              |                    | 50                       | 459.2                                | 56.8                                  | 128       |
|                                                                                            |             |              |                    | 25                       | 454.8                                | 56.4                                  | 121       |
|                                                                                            |             |              |                    | 0                        | 451.2                                | 60.3                                  | 109       |
| I                                                                                          | F1          | E4           | 0.09               | 100                      | 465.1                                | 55.2                                  | 143       |
|                                                                                            |             |              |                    | 75                       | 463.7                                | 53.3                                  | 139       |
|                                                                                            |             |              |                    | 50                       | 461.6                                | 48.3                                  | 129       |
|                                                                                            |             |              |                    | 25                       | 457.7                                | 41.6                                  | 118       |
|                                                                                            |             |              |                    | 0                        | 450.2                                | 32.7                                  | 88        |
| I                                                                                          | F3          | E1           | 0.09               | 100                      | 465.8                                | 50.1                                  | 106       |
|                                                                                            |             |              |                    | 75                       | 460.5                                | 54.3                                  | 116       |
|                                                                                            |             |              |                    | 50                       | 457.2                                | 57.5                                  | 117       |
|                                                                                            |             |              |                    | 25                       | 454.1                                | 58.7                                  | 114       |
|                                                                                            |             |              |                    | 0                        | 450.9                                | 58.6                                  | 108       |
| I                                                                                          | F4          | E1           | 0.08               | 100                      | 464.1                                | 54.2                                  | 138       |
|                                                                                            |             |              |                    | 75                       | 461.9                                | 54.5                                  | 136       |
|                                                                                            |             |              |                    | 50                       | 458.0                                | 53.6                                  | 130       |
|                                                                                            |             |              |                    | 25                       | 453.4                                | 54.4                                  | 123       |
|                                                                                            |             |              |                    | 0                        | 450.9                                | 58.6                                  | 108       |

\*% A is defined as  $100 - (\% T + k)$ , where % T is Beers's Law percent Transmittance, as is well-known in the art, and k represents the light losses due to scattering and reflectance. The scale is from 0 to 100, where higher numbers indicate more light absorption

This emulsion is predominantly AgCl, so that the structural requirement for the practice of the invention is much more stringent than when the substrate is predominantly AgBr. In particular, (a) where dyes may bear two 5 position substituents, at least one of them must be aromatic, and (b) the symmetrical dinaphthoxazole chromophore is excluded from the invention because it does not aggregate on the AgCl emulsion.

It is readily apparent that the above data indicates that the inventive pairs of dyes maintain the height of the combined aggregate peak, that they result in a steady progression of peak wavelength between the long and the short dye, and that they preserve photographic speed, and that all three of

these features are accomplished to a much greater extent than for the comparative pairs of dyes.

## EXAMPLE 2

In this example a predominantly AgBr three-dimensional emulsion of cubic morphology was used.

The nominal halide composition was  $\text{AgBr}_{97.4\%} \text{I}_{2.6\%}$ . The median grain size was  $0.20 \mu\text{m}$  equivalent spherical diameter (esd). The emulsion was chemically sensitized by melting the emulsion and applying the chemical sensitizers NaSCN at a level of 44 mg per mole of silver,  $\text{Na}_2\text{S}_2\text{O}_3 \cdot 5\text{H}_2\text{O}$  at a level of 33 mg per mole of silver, and  $\text{KAuCl}_4$  at a level of 6.6 mg per silver mole.

The sensitizing dyes were added by re-melting the emulsion at 40 degrees C., and adding the dyes from methanolic solutions at a concentration of 0.00035 moles per liter to produce a dye-to-silver ratio of  $8 \times 10^{-4}$  moles of dye per silver mole. The emulsion was held with stirring for 20 minutes, then chilled with stirring.

The two dyes comprising a particular combination were tested by adding each of them individually to the emulsion, and also by adding them to the emulsion simultaneously from pre-mixed co-solutions in the percentages 75% Dye 1, 25% Dye 2; 50% Dye 1, 50% Dye 2; 25% Dye 1, 75% Dye 2.

The cubic emulsion melts were coated on a machine equipped with an extrusion device to deliver the melted emulsion as a single layer to ESTAR™ support. The melts were coated at  $10.8 \text{ mg/dm}^2$  silver and  $77 \text{ mg/dm}^2$  gelatin, and hardened with 0.08% bis(vinylsulfonyl)methylether (BVSME).

A spectrum was obtained of the coated material using a scanning spectrophotometer equipped with an integrating sphere. The coated materials were exposed with a single-grating transmission sensitometer which produces a separate D log E curve at 10 nm intervals across the visible spectrum. The result is a "wedge spectrograph", which is well-known in the art. (See, for example, "Use of Spectral Sensitizing Dyes To Estimate Effective Energy Levels of Silver Halide Substrates", by P. B. Gilman, Jr., in *Photographic Science and Engineering*, Volume 18, Number 5, September/October 1974.) The exposed coatings were processed at 35 degrees C. in an Eastman KODAK RP X-OMAT™ machine.

The data from this experiment for a variety of inventive and comparative dye pairs is shown in Table II.

TABLE II

Data Obtained for Pairs of Dyes on AgBr Cubic Emulsion.  
I = inventive. C = comparative.

| 55 | Type | Long<br>Dye | Short<br>Dye | $\Delta E$<br>(eV) | Ratio<br>(% long<br>dye) | Aggregate<br>Wave-<br>length<br>(nm) | Aggregate<br>Peak<br>Height<br>(% A)* | Speed** |
|----|------|-------------|--------------|--------------------|--------------------------|--------------------------------------|---------------------------------------|---------|
|    |      |             |              |                    |                          |                                      |                                       |         |
| I  | F1   | E1          | 0.08         | 100                | 464.3                    | 57.1                                 | 248                                   |         |
|    |      |             |              | 75                 | 461.6                    | 55.2                                 | 245                                   |         |
|    |      |             |              | 50                 | 457.7                    | 53.4                                 | 241                                   |         |
|    |      |             |              | 25                 | 453.7                    | 54.9                                 | 245                                   |         |
|    |      |             |              | 0                  | 451.1                    | 56.8                                 | 247                                   |         |
| I  | F3   | E1          | 0.09         | 100                | 465.6                    | 57.3                                 | 247                                   |         |
|    |      |             |              | 75                 | 461.6                    | 54.8                                 | 237                                   |         |
|    |      |             |              | 50                 | 457.4                    | 55.4                                 | 240                                   |         |
|    |      |             |              | 25                 | 454.1                    | 56.1                                 | n.a.***                               |         |
|    |      |             |              | 0                  | 451.1                    | 56.8                                 | 244                                   |         |
| 65 | I    | D1          | C1           | 0.05               | 100                      | 441.0                                | 62.0                                  | 224     |
|    |      |             |              |                    | 75                       | 439.7                                | 59.7                                  | 222     |

TABLE II-continued

| Data Obtained for Pairs of Dyes on AgBr Cubic Emulsion.<br>I = inventive. C = comparative. |             |              |                    |                          |                                      |                                       |           |
|--------------------------------------------------------------------------------------------|-------------|--------------|--------------------|--------------------------|--------------------------------------|---------------------------------------|-----------|
| Type                                                                                       | Long<br>Dye | Short<br>Dye | $\Delta E$<br>(eV) | Ratio<br>(% long<br>dye) | Aggregate<br>Wave-<br>length<br>(nm) | Aggregate<br>Peak<br>Height<br>(% A)* | Speed**   |
|                                                                                            |             |              |                    |                          |                                      |                                       |           |
| I                                                                                          | C1          | B1           | 0.06               | 100                      | 433.7                                | 54.0                                  | 218       |
|                                                                                            |             |              |                    | 75                       | 432.9                                | 59.4                                  | 220       |
|                                                                                            |             |              |                    | 50                       | 430.2                                | 60.1                                  | 222       |
|                                                                                            |             |              |                    | 25                       | 427.5                                | 62.9                                  | 225       |
|                                                                                            |             |              |                    | 0                        | 425.0                                | 65.6                                  | 229       |
|                                                                                            |             |              |                    | 100                      | 425.1                                | 65.9                                  | 229       |
| I                                                                                          | B1          | A1           | 0.08               | 75                       | 423.6                                | 64.5                                  | 227       |
|                                                                                            |             |              |                    | 50                       | 419.1                                | 63.1                                  | 222       |
|                                                                                            |             |              |                    | 25                       | 414.1                                | 65.7                                  | 226       |
|                                                                                            |             |              |                    | 0                        | 413.4                                | 68.8                                  | 239       |
|                                                                                            |             |              |                    | 100                      | 467.4                                | 59.2                                  | 250       |
|                                                                                            |             |              |                    | 75                       | 465.0                                | 54.1                                  | 240       |
| C                                                                                          | F1          | C1           | 0.21               | 50                       | 462 & 433                            | 45 & 48                               | 227 & 215 |
|                                                                                            |             |              |                    | 25                       | 460 & 434                            | 35 & 53.6                             | 208 & 217 |
|                                                                                            |             |              |                    | 0                        | 433.6                                | 54.2                                  | 218       |
|                                                                                            |             |              |                    | 100                      | 467.4                                | 59.3                                  | 250       |
|                                                                                            |             |              |                    | 75                       | 464.6                                | 52.5                                  | 244       |
|                                                                                            |             |              |                    | 50                       | 460.8                                | 44.7                                  | 233       |
| C                                                                                          | F1          | A1           | 0.35               | 25                       | 455 & 411                            | 34 & 62                               | 220 & 226 |
|                                                                                            |             |              |                    | 0                        | 413.5                                | 68.9                                  | 238       |

\*% A is defined as  $100 - (\% T + k)$ , where % T is Beers's Law percent Transmittance, as is well-known in the art, and k represents the light losses due to scattering and reflectance. The scale is from 0 to 100, where higher numbers indicate more light absorption.

\*\*n.a. = not available

It is readily apparent that the above data indicates that the inventive pairs of dyes maintain the height of the combined aggregate peak, that they result in a steady progression of peak wavelength between the long and the short dye, and that they preserve photographic speed, and that all three of these features are accomplished to a much greater extent than for the comparative pairs of dyes.

#### EXAMPLE 3

In this example a predominantly AgBr three-dimensional emulsion of octahedral morphology was used.

The nominal halide composition was  $\text{AgBr}_{97.0\%} \text{I}_{3.0\%}$ . The median grain size was  $0.30 \mu\text{m}$  equivalent spherical diameter (esd). The emulsion was chemically sensitized by melting the emulsion and applying the chemical sensitizers  $\text{NaSCN}$  at a level of 150 mg per mole of silver,  $\text{Na}_2\text{S}_2\text{O}_3 \cdot 5\text{H}_2\text{O}$  at a level of 8 mg per mole of silver, and  $\text{KAuCl}_4$  at a level of 5 mg per silver mole.

The cubic emulsion melts were coated on a machine equipped with an extrusion device to deliver the melted emulsion as a single layer to ESTAR<sup>TM</sup> support. The melts were coated at  $21.5 \text{ mg/dm}^2$  silver and  $86 \text{ mg/dm}^2$  gelatin, and hardened with 0.08% bis(vinylsulfonyl)methylether (BVSME).

The sensitizing dyes were added by re-melting the emulsion at 40 degrees C., and adding the dyes from methanolic solutions at a concentration of 0.00032 moles per liter to produce a dye-to-silver ratio of  $4.0 \times 10^{-4}$  moles of dye per silver mole. The emulsion was held with stirring for 20 minutes, then chilled with stirring.

The two dyes comprising a particular combination were tested by adding each of them individually to the emulsion, and also by adding them to the emulsion simultaneously

from pre-mixed co-solutions in the percentages 75% Dye 1, 25% Dye 2; 50% Dye 1, 50% Dye 2; 25% Dye 1, 75% Dye 2.

A spectrum was obtained of the coated material using a scanning spectrophotometer equipped with an integrating sphere. The coated materials were exposed with a single-grating transmission sensitometer which produces a separate D log E curve at 10 nm intervals across the visible spectrum. The result is a "wedge spectrograph", which is well-known in the art. (See, for example, "Use of Spectral Sensitizing Dyes To Estimate Effective Energy Levels of Silver Halide Substrates", by P. B. Gilman, Jr., in Photographic Science and Engineering, Volume 18, Number 5, September/October 1974.) The exposed coatings were processed at 35 degrees C. in an Eastman KODAK RP X-OMAT<sup>TM</sup> machine.

The data from this experiment for a variety of inventive and comparative dye pairs is shown in Table III.

TABLE III

| Data Obtained for Pairs of Dyes on AgBr Octahedral Emulsion.<br>I = inventive. C = comparative. |             |              |                    |                          |                                      |                                       |         |
|-------------------------------------------------------------------------------------------------|-------------|--------------|--------------------|--------------------------|--------------------------------------|---------------------------------------|---------|
| Type                                                                                            | Long<br>Dye | Short<br>Dye | $\Delta E$<br>(eV) | Ratio<br>(% long<br>dye) | Aggregate<br>Wave-<br>length<br>(nm) | Aggregate<br>Peak<br>Height<br>(% A)* | Speed** |
|                                                                                                 |             |              |                    |                          |                                      |                                       |         |
| I                                                                                               | F1          | E1           | 0.06               | 100                      | 460.6                                | 61.6                                  | 257     |
|                                                                                                 |             |              |                    | 75                       | 458.2                                | 60.6                                  | 253     |
|                                                                                                 |             |              |                    | 50                       | 455.2                                | 60.1                                  | 252     |
|                                                                                                 |             |              |                    | 25                       | 452.3                                | 60.9                                  | 253     |
|                                                                                                 |             |              |                    | 0                        | 450.1                                | 62.7                                  | 255     |
|                                                                                                 |             |              |                    | 100                      | 466.6                                | 60.9                                  | 255     |
| I                                                                                               | F3          | E1           | 0.10               | 75                       | 458.5                                | 60.2                                  | 253     |
|                                                                                                 |             |              |                    | 50                       | 454.6                                | 61.7                                  | 254     |
|                                                                                                 |             |              |                    | 25                       | 452.1                                | 62.0                                  | 255     |
|                                                                                                 |             |              |                    | 0                        | 450.1                                | 62.7                                  | 255     |
|                                                                                                 |             |              |                    | 100                      | 460.8                                | 61.0                                  | 257     |
|                                                                                                 |             |              |                    | 75                       | 458.9                                | 59.7                                  | 255     |
| I                                                                                               | F1          | E5           | 0.05               | 50                       | 456.4                                | 58.6                                  | 253     |
|                                                                                                 |             |              |                    | 25                       | 454.0                                | 59.9                                  | 256     |
|                                                                                                 |             |              |                    | 0                        | 452.8                                | 58.2                                  | 262     |
|                                                                                                 |             |              |                    | 100                      | 460.8                                | 61.0                                  | 257     |
|                                                                                                 |             |              |                    | 75                       | 457.6                                | 58.2                                  | 255     |
|                                                                                                 |             |              |                    | 50                       | 451 & 435                            | 56 & 60                               | 250     |
| C                                                                                               | F1          | D2           | 0.15               | 25                       | 435.2                                | 60.2                                  | 244     |
|                                                                                                 |             |              |                    | 0                        | 436.0                                | 64.3                                  | 245     |

\*% A is defined as  $100 - (\% T + k)$ , where % T is Beers's Law percent Transmittance, as is well-known in the art, and k represents the light losses due to scattering and reflectance. The scale is from 0 to 100, where higher numbers indicate more light absorption.

It is readily apparent that the above data indicates that the inventive pairs of dyes maintain the height of the combined aggregate peak, that they result in a steady progression of peak wavelength between the long and the short dye, and that they preserve photographic speed, and that all three of these features are accomplished to a much greater extent than for the comparative pairs of dyes.

#### EXAMPLE 4

The emulsion used was a predominantly silver chloride, ruthenium doped, (1.0.0) tabular emulsion.

The average grain diameter was 0.60 microns equivalent circular diameter (ecd). The average grain thickness was 0.17 microns.

The precise halide ratio was 99.404% chloride and 0.596% iodide. The emulsion was doped with 125 pmm ruthenium hexacyanide.

#### Sensitization

The emulsion was heated to 39° C. and the following additions were made at the rate of mg per silver mole. 50 mg

## 31

of potassium bromide, 1.7 mg of potassium tetrachloroaurate, sensitizing dyes F2 and E1 in amounts shown in Table V, and 3.4 mg of sodium thiosulfate. The emulsion was heated to 60° C., held for 25 min. and then cooled to 39° C. 100 mg of 1-(3-acetamidophenyl)-5-mercaptopotetrazole was added. The emulsion was then coated on triacetate film with the yellow coupler of formula Y—C. The film was then dried.



## Testing

The film was exposed to white light at 3000K for a time of 0.004 sec. It was then processed in the ECP-2™ process for 3 min. at 98° F. The spectral absorption of the coated film samples was measured on a spectrophotometer. Results were obtained for the different levels of sensitizing dyes. These results are given in Table IV.

TABLE IV

| Sample Number | F2 quantity | E1 quantity | Minimum density | Speed** | Aggregate Wavelength (nm) | Aggregate Peak Height (% A)* |
|---------------|-------------|-------------|-----------------|---------|---------------------------|------------------------------|
| 5-1           | 100         | 0           | 0.15            | 168     | 471                       | 30.8                         |
| 5-2           | 83.5        | 16.5        | 0.12            | 190     | 469                       | 29.0                         |
| 5-3           | 67.0        | 33.0        | 0.11            | 172     | 468                       | 26.1                         |
| 5-4           | 58.7        | 41.3        | 0.10            | 167     | 466                       | 25.8                         |
| 5-5           | 50.3        | 49.7        | 0.08            | 164     | 462                       | 24.8                         |
| 5-6           | 42.0        | 58.0        | 0.10            | 166     | 461                       | 22.3                         |
| 5-7           | 33.7        | 66.3        | 0.10            | 169     | 459                       | 25.1                         |
| 5-8           | 16.8        | 83.2        | 0.09            | 160     | 458                       | 27.3                         |
| 5-9           | 0           | 100         | 0.08            | 156     | 456                       | 30.6                         |

\*% A is defined as  $100 - (\% T + k)$ , where % T is Beers's Law percent Transmittance, as is well known in the art, and k represents the light losses due to scattering and reflectance.

\*\*The speed is reported on a scale of 0 to 100, where higher numbers indicated more light absorption.

The dye quantities given are the percent ratios of the millimoles of dye per silver mole. As can be seen, the dye peak transitions smoothly from 471 nm to 456 nm as the ratio of dye changes.

## EXAMPLE 5

Dye combination (Table V) were made from two dyes (Table B) which were blended in the following ratios 75/225, 50/50 and 25/5. Dyes and dye combination at a level of  $3.8 \times 10^{-4}$  moles/Ag mole, were added to an aurous sulfide sensitized  $0.39 \mu\text{m}$  (cubic edge length) silver chloride cubic emulsions which had 1.0% bromide present. The emulsions were coated on a polyester support in a Black and White

## 32

format. The coatings were given a  $1/10$  second exposure on a wedge spectrographic instrument covering a wavelength range from 350 to 750 nm. The instrument contains a tungsten light source and a step tablet ranging in density from 0 to 3 density steps. Correction for the instrument's variation in spectral irradiance with wavelength is done via computer. Results are reported in Table V. Delta is the speed of a coating at a Dye 1/Dye 2 ratio of 25/75 minus the speed

## Y-C

Y-C

## Processing

Temperature 68° F. (20° C.)

35

|    | Chemical        | Process time          |
|----|-----------------|-----------------------|
| 40 | DK-50 developer | 6 minutes 0 seconds   |
|    | Stop bath*      | 15 seconds            |
|    | Fix**           | 5 minutes 0 seconds   |
|    | Wash            | 10 minutes 0 seconds. |

\*composition is 128 mL acetic acid diluted to 8 L with distilled water.  
\*\* composition is 15.0 g sodium sulfite, 240.0 g sodium thiosulfate, 13.3 mL glacial acetic acid, 7.5 g boric acid, and 15.0 g potassium aluminum sulfate diluted to 1.0 L with distilled water.

## TABLE V

| 50         | Data comparing change in photographic speed |       |                 |                                    |       |       |       |       |         |
|------------|---------------------------------------------|-------|-----------------|------------------------------------|-------|-------|-------|-------|---------|
|            | I = inventive. C = comparative.             |       |                 |                                    |       |       |       |       |         |
| Sample No. | Dye 1                                       | Dye 2 | $\Delta E$ (eV) | $\lambda_{max}$ (nm) of Dye blends |       |       |       |       | Del-ta* |
|            |                                             |       |                 | 100/0                              | 75/25 | 50/50 | 25/75 | 0/100 |         |
| 5-I-1      | F2                                          | E1    | 0.11            | 470                                | 467   | 462   | 455   | 451   | -5      |
| 5-I-2      | F1                                          | E1    | 0.08            | 465                                | 462   | 459   | 455   | 451   | -8      |
| 5-I-3      | F4                                          | E1    | 0.08            | 464                                | 462   | 458   | 453   | 451   | -6      |
| 5-I-4      | F2                                          | F8    | 0.03            | 470                                | 469   | 466   | 464   | 464   | -4      |
| 5-I-5      | F2                                          | F9    | 0.05            | 470                                | 469   | 467   | 465   | 462   | 2       |
| 5-I-6      | F2                                          | F6    | 0.06            | 470                                | 467   | 464   | 462   | 459   | -1      |
| 5-I-7      | F2                                          | F10   | 0.08            | 470                                | 467   | 464   | 460   | 456   | -3      |
| 5-I-8      | F2                                          | E2    | 0.08            | 470                                | 468   | 465   | 461   | 457   | -4      |
| 5-I-9      | F2                                          | E6    | 0.07            | 470                                | 468   | 465   | 461   | 458   | -10     |
| 5-I-10     | F2                                          | E'1   | 0.10            | 470                                | 467   | 463   | 456   | 453   | -7      |
| 5-I-11     | F2                                          | E'2   | 0.12            | 470                                | 467   | 462   | 454   | 450   | -8      |
| 5-I-12     | F1                                          | E3    | 0.08            | 465                                | 464   | 461   | 456   | 452   | -11     |
| 5-I-13     | F1                                          | E4    | 0.09            | 465                                | 464   | 462   | 458   | 450   | -18     |
| 5-I-14     | F3                                          | E1    | 0.09            | 466                                | 461   | 457   | 454   | 451   | -1      |

TABLE V-continued

| Sample No. | Dye 1 | Dye 2 | AE (eV) | λ <sub>max</sub> (nm) of Dye blends |       |       |       |       | Delta ta* |
|------------|-------|-------|---------|-------------------------------------|-------|-------|-------|-------|-----------|
|            |       |       |         | 100/0                               | 75/25 | 50/50 | 25/75 | 0/100 |           |
| 5-I-16     | F2    | F7    | 0.06    | 470                                 | 468   | 466   | 464   | 460   | 0         |
| 5-C-1      | F1    | D1    | 0.16    | 465                                 | 462   | 459   | 440   | 439   | -30       |

\*Delta is the speed of a coating at a Dye 1/Dye 2 ratio of 25/75 minus the speed at a Dye 1/Dye 2 ratio of 75/25.

As can be seen from Table V, the invention dye combinations allow the sensitization maximum to be adjusted by varying the ratio of the two dyes. The invention dye combinations give less speed loss than the comparison dye combination.

#### EXAMPLE 6

##### Invention

The emulsion (invention) is precipitated by bringing together NaCl and AgNO<sub>3</sub>, in the presence of gelatin, antifoamant, dithio-3,6-octane-1,8-diol, and glutaryl diamino phenyldisulfide to form grains of cubic edge length 0.5 μm–0.8 μm, with an aspect ratio of 1.2 or less. After desalting, the emulsion is then chemically and spectrally sensitized by the addition of ortho-succinamidophenyldisulfide, gold(I) bis(1,4,5-trimethyl-1,2,4-triazolium-3-thiolate)gold(I) fluoroborate, Dye F2, Dye E1 and sodium thiosulfate followed by a heat cycle.

After the heat cycle, these three chemicals are added in any sequence: 1-(3-acetamidophenyl)-5-mercaptopotetrazole at about 70 mg/Ag mol, and potassium bromide 0.005 mol bromide/mol Ag.

##### Check

The emulsion (check) is precipitated by bringing together NaCl and AgNO<sub>3</sub>, in the presence of gelatin antifoamant, dithio-3,6-octane-1,8-diol, nitric acid, and Hg to form gains of cubic edge length 0.0 μm–0.8 μm. The emulsion is then finished by addition of iridium (K<sub>2</sub>IrCl<sub>6</sub>), sulfur gold(I)/sulfur compound (AuO<sub>6</sub>S<sub>4</sub>·2H<sub>2</sub>O·3Na, 1-(3-acetamidophenyl)-5-mercaptopotetrazole, and thiourea, followed by a heat cycle, followed by addition of comparative dye COMP-1, 1-(3-acetamidophenyl)-5-mercaptopotetrazole, KBr, and gelatin.



In the check emulsion, some of the dye COMP-1 crystallizes making it necessary to filter the emulsion before storage and/or use. Further excess dye is needed to compensate for the dye that crystallizes out of the emulsion.

In the inventive emulsion, the dye combination of dye F2 (having a λ<sub>max</sub> of 470 nm) and dye E1 (having a λ<sub>max</sub> of 452 nm) does not crystallize in solution, in the sensitized emulsion. Spectroscopic analysis of the emulsions have

shown there to be no free dye. Therefore, no filtering is required of the emulsion prior to storage. Dyes F2 and E1 are fully incorporated into the emulsion.

To illustrate that the new emulsion provides the same sensitometric performance as the check emulsion, the new emulsion was evaluated in the multilayer format shown in Table V.

TABLE VI

##### Multilayer Coating Format

|                                |  |
|--------------------------------|--|
| Layer 1: Antihalation Layer    |  |
| Layer 2: Blue Sensitive Layer  |  |
| Gelatin                        |  |
| Silver                         |  |
| Y-1                            |  |
| Dibutyl phthalate              |  |
| UV-1                           |  |
| Layer 3: Interlayer            |  |
| Gelatin                        |  |
| SC-1                           |  |
| SF-1                           |  |
| Layer 4: Red Sensitive Layer   |  |
| Gelatin                        |  |
| Silver                         |  |
| C-1                            |  |
| Tritolyl phosphate             |  |
| Tris(2-ethylhexyl phosphate)   |  |
| SC-1                           |  |
| Layer 5: Interlayer            |  |
| Gelatin                        |  |
| SC-1                           |  |
| SF-1                           |  |
| Layer 6: Green Sensitive Layer |  |
| Gelatin                        |  |
| Silver                         |  |
| M-1                            |  |
| Tritolyl phosphate             |  |
| SC-1                           |  |
| Layer 7: Overcoat              |  |

Y-1 =



UV-1 =



SC-1 = 1,4-isododecyl hydroquinone

SF-1 =



TABLE VI-continued

| Multilayer Coating Format |                                                                                   |
|---------------------------|-----------------------------------------------------------------------------------|
| C-1 =                     |  |
| M-1 =                     |  |

Film samples were given white light exposures and processed in Kodak's ECP-2B process, which is well-known in the trade and is documented in Kodak's H-24 manual. The results are given in Table VI(a).

TABLE VI(a)

| CHARACTERISTIC                     | Emulsion performance characteristics             |                                                  |
|------------------------------------|--------------------------------------------------|--------------------------------------------------|
|                                    | CHECK<br>EMULSION                                | INVENTION EMULSION                               |
| Wasted dye due to crystals         | 30%                                              | none                                             |
| Organic solvents speed             | yes<br>100                                       | none<br>100                                      |
| contrast                           | 1.0                                              | 1.0                                              |
| short-term LIK                     | <0.01 logE speed change per 1.0 log 10 (minutes) | <0.01 logE speed change per 1.0 log 10 (minutes) |
| raw stock keeping                  | no change 3 months/ 13° C.                       | no change 3 months/ 13° C.                       |
| lambda-max                         | 461 nm                                           | 466 nm                                           |
| High intensity reciprocity failure | no change<br>1/2000"-1/100"                      | no change 1/2000"-1/100"                         |
| sulfur:gold molar ratio            | 2:1 minimum                                      | unrestricted                                     |

The invention has been described in detail with particular reference to preferred embodiments, but it will be understood that variations and modifications can be effected within the spirit and scope of the invention.

What is claimed is:

1. A photographic element comprising at least one silver halide emulsion layer in which:
  - a) the silver halide has been sensitized with a first J-aggregating blue sensitizing dye having a  $\lambda_1$  less than or equal to about 475 nm and a second J-aggregating blue sensitizing dye having a  $\lambda_2$ , wherein said first and second dyes form a mixed aggregate and wherein  $\lambda_1$  is longer than  $\lambda_2$ , and  $\lambda_1$  and  $\lambda_2$  are separated by an

energy gap,  $\Delta E$ , which does not exceed 0.12 eV, where  $\Delta E$  is defined by the following equation:

$$\Delta E = 1.25(\text{nm})(\text{eV}) \times 10^3 \left[ \frac{1}{\lambda_2(\text{nm})} - \frac{1}{\lambda_1(\text{nm})} \right] \leq 0.12(\text{eV})$$

wherein  $\lambda_1$  is the wavelength in nanometers ( $\mu\text{m}$ ) of maximum absorption of a silver halide emulsion sensitized with the long dye and  $\lambda_2$  is the wavelength of maximum absorption of a silver halide emulsion sensitized with the short dye, with the proviso that neither the first nor the second dye contains selenium and that each dye contains an anionic water solubilizing group; and

15 b) the silver halide has been chemically sensitized with a gold(I) compound of formula (Ia) or (Ib):



20 or



wherein

25 L is a mesoionic compound;

X is an anion; and

$\text{L}^1$  is a Lewis donor ligand.

2. A photographic element according to claim 1, wherein the emulsion layer further comprises a disulfide compound of formula (II):



45 wherein:

X' is independently  $-\text{O}-$ ,  $-\text{NH}-$  or  $-\text{NR}-$ , where R is an alkyl group, a fluoroalkyl group, an aryl group or a sulfonyl group;

40 m and r are independently 0, 1 or 2, with the proviso that m and r are not both 0;

M is  $-\text{H}$  or a cationic species;

Ar is an aromatic group; and

$\text{L}^2$  is a linking group, where p is 1.

55 3. A photographic element according to claim 1, wherein L is a mesoionic compound represented by the formula:



wherein a, b, c, d, and e represent the unsubstituted or substituted atoms necessary to complete a heterocyclic ring; the circle with the + sign on the heterocyclic ring symbolizes six delocalized  $\pi$  electrons associated with a partial positive charge on the heterocyclic ring.

4. A photographic element according to claim 3, wherein the mesoionic heterocyclic ring is a triazolium or tetrazolium 5-membered ring.

5. A photographic element according to claim 1, wherein the gold (I) compound is of the formula:



wherein R<sub>6</sub>, R<sub>7</sub>, and R<sub>8</sub> are independently a substituted or unsubstituted alkyl group, a substituted or unsubstituted alkenyl group, an amino group, a substituted or unsubstituted aryl group, and X<sup>-</sup> is a halogen or BF<sub>4</sub><sup>-</sup> anion.

6. A photographic element according to claim 1, wherein the gold (I) compound is of the formula:



wherein R<sub>6</sub> and R<sub>7</sub> are independently a substituted or unsubstituted alkyl group, a substituted or unsubstituted alkenyl group, an amino group, a substituted or unsubstituted aryl group, and X<sup>-</sup> is a halogen or BF<sub>4</sub><sup>-</sup> anion.

7. A photographic element according to claim 1, wherein the gold (I) compound is of the formula:



wherein R<sub>6</sub>, R<sub>7</sub>, R<sub>8</sub>, and R<sub>9</sub> are independently a substituted or unsubstituted alkyl group, a substituted or unsubstituted alkenyl group, an amino group, a substituted or unsubstituted aryl group, and X<sup>-</sup> is a halogen or BF<sub>4</sub><sup>-</sup> anion.

8. A photographic element according to claim 1, wherein the silver halide emulsion layer further comprises a disulfide compound represented by formula (II):

(II)



wherein:

20 X' is independently —O—, —NH— or —NR—, where R is an alkyl group, a fluoroalkyl group, an aryl group or a sulfonyl group;

25 m and r are independently 0, 1 or 2, with the proviso that m and r are not both 0;

M is —H or a cationic species;

Ar is an aromatic group;

p is 0 or 1; and

30 L<sup>2</sup> is a linking group, where p is 1.

35 9. A photographic element according to claim 1, wherein the disulfide compound is of the formula:



40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665

39



wherein  $Z_1$ ,  $Z_2$  and  $Z''$  are independently a hydrogen or halogen atom or a substituted or unsubstituted alkyl, substituted or unsubstituted alkoxy, substituted or unsubstituted aromatic and substituted or unsubstituted heterocyclic group; and  $R_1$  and  $R_2$ , are independently substituted or unsubstituted alkyl, substituted or unsubstituted alkenyl or substituted or unsubstituted aryl, with the proviso that for each dye at least one of  $R_1$  and  $R_2$  contains an anionic solubilizing group.

11. A photographic element according to claim 10, wherein the first dye has a peak wavelength of about 470 nm and the second dye has a peak wavelength of about 450 nm.

12. A photographic element according to claim 10, wherein the first dye has a peak wavelength of about 450 nm and the second dye has a peak wavelength of about 440 nm.

13. A photographic element according to claim 10, wherein the first dye has a peak wavelength of about 420 nm and the second dye has a peak wavelength of about 410 nm.

14. A photographic element according to claim 10, wherein the first dye is of the structure:



and the second dye is of the structure:



wherein  $Z_1$  and  $Z_2$  are independently a hydrogen or halogen atom or a substituted or unsubstituted alkyl, substituted or unsubstituted alkoxy, substituted or unsubstituted aromatic,

40

substituted or unsubstituted alkoxy carbonyl and substituted or unsubstituted heterocyclic group; and  $R_1$  and  $R_2$ , are independently substituted or unsubstituted alkyl, substituted or unsubstituted alkenyl or substituted or unsubstituted aryl.

15. A photographic element according to claim 10, wherein the first dye is of the structure:



and the second dye is of the structure:



wherein  $Z_1$ ,  $Z_2$  and  $Z''$  are independently a hydrogen or halogen atom or a substituted or unsubstituted alkyl, substituted or unsubstituted alkoxy, substituted or unsubstituted aromatic, substituted or unsubstituted alkoxy carbonyl and substituted or unsubstituted heterocyclic group; and  $R_1$  and  $R_2$ , are independently substituted or unsubstituted alkyl, substituted or unsubstituted alkenyl or substituted or unsubstituted aryl.

16. A photographic element according to claim 10, wherein the first dye is of the structure:



and the second dye is of the structure:



wherein  $Z_1$  and  $Z''$  are independently a hydrogen or halogen atom or a substituted or unsubstituted alkyl, substituted or unsubstituted alkoxy, substituted or unsubstituted aromatic, substituted or unsubstituted alkoxy carbonyl and substituted or unsubstituted heterocyclic group; and  $R_1$  and  $R_2$ , are independently substituted or unsubstituted alkyl, substituted or unsubstituted alkenyl or substituted or unsubstituted aryl.

17. A photographic element according to claim 10, wherein the first dye is of the structure:

41



and the second dye is of the structure:



wherein Z<sub>1</sub> and Z<sub>2</sub> are independently a hydrogen or halogen atom or a substituted or unsubstituted alkyl, substituted or unsubstituted alkoxy, substituted or unsubstituted aromatic, substituted or unsubstituted alkoxy carbonyl and substituted or unsubstituted heterocyclic group; and R<sub>1</sub> and R<sub>2</sub>, are independently substituted or unsubstituted alkyl, substituted or unsubstituted alkenyl or substituted or unsubstituted aryl.

**18.** A photographic element according to claim 1, wherein said first dye and/or said second dye is of structure I:



6,140,035  
42

wherein:

5 Z<sub>1</sub> is phenyl, pyrrolyl, furanyl, thieryl, alkoxy carbonyl or a fused benzene ring;

Z<sub>2</sub> is phenyl, pyrrolyl, furanyl, thieryl, alkoxy carbonyl or halogen, R<sub>1</sub> and R<sub>2</sub> are acid substituted alkyl groups; and

10 A<sup>+</sup> is a counterion.

**19.** A photographic element according to claim 1, wherein said first and/or said second dye is of structure II:



20 25 wherein

X is O or S,

Y<sub>1</sub> is pyrrolyl, furanyl, thieryl, alkoxy carbonyl or phenyl;

Y<sub>2</sub> is a 4,5-benzo substituent when X is O and a phenyl carbamoyl or a phenylcarboxamido substituent when X is S;

30 35 R<sub>3</sub> and R<sub>4</sub> are acid substituted alkyl groups; and

B<sup>+</sup> is a counterion.

\* \* \* \* \*